# EUROPEAN PATENT SPECIFICATION

(11) **EP 4 204 618 B1**
(45) Date of publication and mention of the grant of the patent: **26.03.2025**
(21) Application number: 21830350.1
(22) Date of filing: 27.08.2021
(51) Int. Cl.: D04H 1/4266, D04H 1/732

(54) **A METHOD FOR PRODUCING A NON-WOVEN TEXTILE, AND A NON-WOVEN TEXTILE**
VERFAHREN ZUR HERSTELLUNG EINES VLIESSTOFFES UND VLIESSTOFF
PROCÉDÉ DE PRODUCTION D'UN TEXTILE NON TISSÉ, ET TEXTILE NON TISSÉ

(30) Priority: 28.08.2020 NL 2026370
(43) Date of publication of application: 05.07.2023
(73) Proprietor: Neffa Holding BV, 3812 PK Amersfoort (NL)
(72) Inventor: HOITINK, Aniela Maria, 3762KG Soest (NL)
(74) Representative: Dogio Patents B.V.
(86) International application number: PCT/NL2021/050524
(87) International publication number: WO 2022/045889

(56) References cited:
- WO-A1-2020/006133
- WO-A1-99/25924
- CA-A1- 2 718 435
- GB-A- 1 535 375

## Description

The present invention relates to a method for producing a non-woven textile.

Non-woven textiles are well known and widely used from disposable diapers and surgery gowns to durable materials for wind stoppers and rain coats.

Non-woven textiles can be produced by various methods, such as a wet-laid method. In a wet-laid method a dispersion of fibers in a dispersion medium is applied to the surface of a support, after which the dispersion medium is eliminated and the fibers form a web. This web conforms to the shape of the support, thus in case of a three-dimensional support of a desired shape, the non-woven textile has said desired shape without cutting and sewing. The non-woven textile may also have a surface structure, for example if an embossed support is used.

Non-woven textiles may be made from a diverse range of materials, such as synthetic fibers including polyethylene, but textiles based on natural materials are desirable, including the characteristic of how they feel to the touch (skin feel).

It is known in the art to make non-woven textiles from biobased fibers, that is fibers from biological (i.e. natural) origin, but they may lack the desired strength and/or durability. In for example WO 2020/006133 A1, a second material, in the form of a woven textile layer, is embedded in a matrix of biobased fibers to provide strength to the biobased fibers. According to WO 2020/006133 A1 however, the biobased fibers in the form of a fungal matrix are grown into the woven textile layer, which is a time-consuming process and difficult to control, and requires the biobased fibers to be alive during production of the non-woven textile.

CA 2,718,435 A1 teaches applying fibers in an isotropic orientation in which the fibers are oriented transverse to a product material. These transversely oriented fibers are intended to provide a specific feel, but do not contribute substantially to the strength the product material, and in particular these fibers do not form a web.

It is the object of the invention to provide a biofiber-based non-woven textile with enhanced strength and/or durability in a simple way without compromising the skin feel.

To this end, according to a first aspect, the invention provides a method which comprises the following steps:
i) applying a layer of a dispersion comprising dispersion medium and biobased first fibers on a support, wherein the biobased first fibers are fibers derived from a micro-organism cultured in a liquid culture medium, and wherein prior to said applying a plasticized has been added to the dispersion;
ii) depositing reinforcing second fibers on the layer of the dispersion, wherein the reinforcing second fibers are separate fibers which are not part of a fabric, and wherein the second fibers have an average length that is at least 10x longer than the average length of the first fibers; and
iii) eliminating the dispersion medium to form the non-woven textile comprising a web of biobased first fibers.

In this way, an enhanced strength is provided to a non-woven textile based on biobased first fibers while
- substantially maintaining the simplicity of the method,
- substantially preserving the skin feel at a side of the non-woven textile facing the support.

The second fibers will typically be applied en masse, for example as a suspension, using a brush or by spraying. In the present application, separate fibers means that they are individual fibers. Thus, they are not part of a fabric, be it woven, non-woven, or a fabric wherein the fibers are interconnected by glue or heat (melting of fibers), or by addition of adhesive or cross-linking agents.

At most, part of the dispersion medium may be eliminated before the second fibers are applied, so as to allow the second fibers to become embedded in a wet matrix of the first fibers. Elimination typically involves drying, e.g. by passing dry air across the surface of the layer of the dispersion, taking care not to blow it away. The air may be heated air. In this way, redistribution or dripping of the dispersion applied in step i) under gravitational force is reduced. Therefore, irregularities formed by for example dripping of the dispersion may be reduced and the production of the non-woven textile at non-horizontal surfaces may be facilitated.

It is known in the art to make a non-woven textile having enhanced strength by chemical treatment or chemical modification of the biobased fibers or non-woven textiles. Such a treatment may take away from the desired properties of the non-woven textile with respect to skin feel. Should the chemical treatment or modification require undesirable use of chemicals, the present invention allows for these to be avoided. The reduction or even elimination of the use of chemicals renders the method more sustainable.

The non-woven textile may be produced without an additional step after step iii) of interconnecting the first fibers after forming of the web. This reduces the work for producing a non-woven textile by avoiding a separate step of chemical bonding, thermal bonding, mechanical bonding or any other step(s) required to link the first fibers to each other.

In the present application, the term biobased first fibers includes refined biobased first fibers such as mycelium, cellulose, etc. but also chemically produced or processed biobased first fibers such as viscose or lyocell.

The first fibers are preferably dispersed in a dispersion medium that is water based. But the dispersion fluid may be any fluid suitable for wet-laid processes and may be based on other volatile liquids, such as alcohols like methanol, ethanol or propanol, any other organic volatile fluid or a combination of these liquids, such as water and ethanol. In this way the elimination of the dispersion medium may be facilitated or the first fibers may be dispersed in the dispersion medium more effectively. Preferably the dispersion medium is non-toxic an/or of natural origin and/or non-harmful to the environment.

The concentration of first fibers in the dispersion is at least 0.1% w/v, preferably at least 5% w/v, more preferably at least 10% w/v and most preferably at least 15% w/v. Preferably, the concentration of the first fibers in the dispersion is below 60% w/v.

In an embodiment, after step iii), the first fibers comprise 20 - 80 % weight of the non-woven textile; the second fibers comprise 1 - 40 % weight of the non-woven textile; and the plasticizer comprises 5 - 50 % weight of the non-woven textile, wherein the combined % weight of the first fibers, the second fibers and the plasticizer is at least 65% of the weight of the non-woven textile, preferably at least 80%; and wherein the %weight of the second fibers is less than the %weight of the first fibers.

Preferably the first fibers are less than 50 micrometer, more preferably less than 25 micrometer, even more preferably less than 15 micrometer and most preferably less than 8 micrometer in diameter. In this way, a face of the web facing the support structure adopts a smooth texture after elimination of the dispersion medium.

The reinforcing second fibers may be fibers with a higher tensile strength than the first fibers. The reinforcing second fibers have an average length that is at least 10x longer than the average length of the first fibers.

Typically, second fibers have a cylindrical cross-section, but may be flattened, curved, bend or in any other elongated form as well. The method may also be performed with second fibers wherein the circumferential surface of the second fibers is microfibrilated. In this way the strength and/or durability of the web may be improved.

The second fibers are preferably less than 100 micrometer in diameter, more preferably in the range of 15 to 50 micrometer. In this way, the second fibers provide strength to the non-woven textile, but also allow for a more homogeneous distribution of the first fibers.

The second fibers are preferably at least 0.3 millimeter, more preferably at least 2 millimeter, even more preferably at least 5 millimeter and most preferably at least 10 millimeter long. In this way, the strength and the durability of the non-woven textile produced according to the method is improved.

In a plane projected parallel to a face of the web, the second fibers typically cover 10% - 90%, preferably 20% - 75%, more preferable 30% - 50% of a total surface of the first fibers lying in the plane.

The second fibers may for example be added by flocking, air laying, fiber spinning or electrospinning. In this way the distribution of second fibers can be controlled precisely, and may the non-woven textile be provided with portions with different properties by the use of different deposit techniques in different portions of the non-woven textile.

The surface of the support may be a flat surface, but may also be a surface of a three dimensional shape or a structured surface. In this way a two dimensional sheet, a three dimensionally shaped web or a web with a structure may be produced. The surface of the support may be provided by the surface of a mold, but can also be the surface of a web formed earlier on a mold, whether or not formed by the method according to the invention. The mold may for example be a torso of a person.

The non-woven textile may be removed from the support, but this is not done in case it is desired to provide a support with a non-woven textile, i.e. the non-woven textile is part of a product. In case the non-woven textile is to be removed from the support, the support will typically have a surface that will help in removal of the textile (chosen not to excessively stick to the textile). In case of a product, the opposite is preferred.

According to a favourable embodiment, the layer of the dispersion in step i) is applied by spraying.

Spraying the dispersion allows for a more controlled application of the layer of the dispersion and the first fibers, resulting in a non-woven textile of higher quality. For example, the risk of formation of air bubbles is smaller, resulting in a more homogeneous and consistent layer of the dispersion and therefore a non-woven textile of higher quality.

According to a favourable embodiment, step i) is preceded by a step comprising
- supplying a dispersion of biobased first fibers, said first fibers being dispersed in a dispersion medium, and
- eliminating at least part of said dispersion medium so as to form a web on the support; which step is performed at least once, and step i) comprises applying the layer of dispersion onto the web.

In this way, a thicker non-woven textile may be made with a well-controlled thickness and the risk of second fibers protruding to the side of the fabric facing the support and thus delamination of the non-woven textile is reduced. The dispersion medium is typically eliminated by evaporation, which may be facilitated using heat and/or supply of drying air.

Furthermore, this embodiment facilitates the manufacturing of a non-woven textile in a non-horizontal orientation, since a stack of relatively thin layers can be applied and dried to obtain the desired thickness of the non-woven textile as opposed to a relatively thick layer being applied in one go. Typically, the step is executed at least 2 times, preferably at least 5 times and more preferable at least 10 times.

According to a favourable embodiment, the method further comprises between steps ii) and iii) a step of applying a further layer of a further dispersion on top of the layer of the dispersion, said further dispersion comprising further dispersion medium and biobased third fibers.

In this way, the method provides for a further web which provides the side of the fabric facing away from the support with a skin feel determined by the biobased third fibers that were applied last.

The strength of the fabric may be improved by better embedding of the second fibers.

The further dispersion medium of the further dispersion may be the same dispersion medium as the dispersion medium, of have a different composition. Furthermore, the biobased third fibers may be the same fibers as the first or second fibers, or may be fibers with different properties, such as antimicrobial or skin-caring properties.

The biobased first fibers are fibers derived from a micro-organism cultured in a liquid culture medium.

This makes it possible to circumvent the production of plant based fibers which typically require large surfaces of land, pesticides, and expensive harvesting followed by extensive processing of fibers. In contrast, growing a micro-organism such as mycelium in a bioreactor can be performed efficiently and the mycelium may be simply harvested (e.g. by filtration) or even as such without a harvesting step and the liquid culture medium is the dispersion medium. Optionally, the mycelium may be diluted or resuspended in dispersion medium (water), and is then ready for forming the non-woven textile.

The micro-organism may for example be a fungus, protozoa, bacteria or algae.

The first fibers may comprise a biobased material derived from: fungal mycelium, yeast, algae, bacteria, cultured animal or plant cells, and fibers derived from animal and/or plant cells cultured in a liquid culture medium. The cultured animal or plant cells may for instance be cultured in a bioreactor.

According to a favourable embodiment, the biobased first fibers are in the form of a biological material chosen from: fungal mycelium, yeast, algae, bacteria, and/or cultured animal or plant cells.

In this way the resources for forming the web are cheap and easy to obtain and may require little production facilities for production.

According to a favourable embodiment, the biobased first fibers are not chemically processed.

In this way, the production of non-woven textiles can occur faster and safer, since a step of chemical treatment or chemical modification is not necessary. Suitable biological materials may be for example harvested fungal mycelium, algae material, bacteria, cultured animal or plant cells, and/or fibers derived from animal and/or plant cells cultured in a liquid culture medium. Biological materials may also be micronized and/or microfibrillated, thereby increasing hairiness of the fibers and enhancing mutual binding capacity.

According to a favourable embodiment, the second fibers are selected from natural fibers, regenerated fibers, recycled fibers, synthetic fibers, functional fibers, or any combination thereof, preferably the second fibers are hydrophilic.

In this way, second fibers may be selected which provide the non-woven textile with desired characteristics. Natural fibers can be used if the non-woven textile needs to be biodegradable and may be derived from plant material, such as wood, grass, leaves, cellulose or from animal material, such as wool, mohair, cashmere, angora, silk, spider silk. However, mineral material such as chrysotile, amosite, crocidolite, tremolite, anthophyllite and actinolite can also be used as second fibers. Preferably, the fibers are natural fibers. Regenerated fibers may be suitable for the same purpose and may be made from materials such as viscose, lyocell, cellulose acetate, Azlon or any other modified cellulose. Furthermore, recycled fibers may be used which are too short for respinning and which would have to be discarded for production of woven fabrics. Synthetic fibers may reduce the cost of the non-woven textile, suitable synthetic fibers may be made from materials such as polypropylene, polyester, elastane, polyvinyl chloride. Special properties like resistance to environmental conditions such as wear, tear and/or higher temperatures may be provided to the non-woven textile by using second fibers made from aramid, liquid-crystal polymers (LCP), carbon, glass, metallic fibers. Fibers with special properties endow the produced non-woven textile with resistance or electrical conductivity, and may thus confer to a user protection or utility of measuring biological functions like heart rate or muscle function. A mixture of fibers of any of these material may be used to confer multiple properties. Hydrophilic fibers provide for better adherence to the first biobased fibers.

According to a favourable embodiment, the second fibers are added isotropically with respect to each other.

An isotropic orientation of the second fibers with respect to each other may for example be achieved by carding the second fibers prior to step ii). The resulting isotropically oriented second fibers may be applied manually or by use of for example a robot in step ii) in a direction parallel to the support. In this way, the isotropic orientation of the second fibers provides an improved strength to the non-woven textile when they are added to the layer of the dispersion.

CA2718435A1 also applies second fibers in an isotropic orientation; however these fibers are oriented transverse to the support and therefore do not contribute substantially to the strength of the non-woven textile.

According to a favourable embodiment, the second fibers are added anisotropically with respect to each other.

This may for example be achieved by electrostatic flocking, wherein an electric charge is applied on the support while adding the second fibers. This results in at least a portion of the second fibers being oriented perpendicularly to the support. After removing the electric charge, at least part of the perpendicularly orientated second fibers will fall over and adopt an orientation parallel to the support but random with respect to each other. This anisotropic orientation may improve the suppleness of the non-woven textile.

A plasticizer is added to the dispersion prior to step i), wherein the plasticizer is preferably a sugar, a sugar alcohol, a polyol, polyolester and/or an alpha hydroxy acid, or a combination thereof, more preferably sorbitol and citric acid. Typically, the resulting non-woven textile has a plasticizer content of between 5 and 50% wt., preferably between 10% and 30% wt.

The addition of the plasticizer may render the obtained non-woven textile more durable. The plasticizer may protect the non-woven textile from becoming brittle, fragile, and/or rigid. Examples of plasticizers are glycols, glyceryl triacetate, polymeric polyols, quillaia, but also complex compositions like honey, molasses, aloe vera, castor oil, glycerides, triglycerides and other mineral or organic oils or any combinations hereof.

According to a favourable embodiment, subsequent to all other steps a step of applying a coating is applied on at least one exposed surface, preferably all exposed surfaces of the non-woven textile.

The coating can for example be a flexible, protecting and/or reinforcing coating. In this way, the durability of the non-woven textile may be improved by retaining dispersion medium and/or retaining the plasticizer in the non-woven textile after consolidation of the web and or further web. The coating may be biologically degradable and/or UV-resistant, and optionally comprise color pigments.

According to a favourable embodiment, the method comprises a step of applying and adhering at least one component to the web.

In this way, additional functionality can be embedded in the non-woven textile. Components like technical components, for example led-lighting, sensors, RFID tags or NFC chips, or embellishments, for example sequins, beads, cord, appliqué and lace, may be directly incorporated without glueing, sewing or without otherwise engaging the component to the non-woven textile reducing the cost and number of steps during production of an enhanced non-woven textile.

According to a favourable embodiment, the method comprises a dyeing step. This step is typically carried out prior to step ii), e.g. by mixing in a dye and/or pigment in the dispersion that is applied in step i).

Preferably in this step, a dye and/or pigment is co-applied with at least one chosen from first and second fibers. In this way, the dye and/or pigment is taken up in the textile together with the fibers, avoiding a separate dyeing step. In particular, no additional liquid may be required to mix the dye and/or pigment into the textile. The dye and/or pigment is embedded in the textile, making the dye of the textile to be less easily damaged while using the textile.

Also, it is no longer necessary to wash the textile to remove surplus dye, which is typically an onerous step in the production of state of the art textiles.

In an embodiment, step ii) is caried out and completed within 2 hours from the start of step i), preferably within 0,5 hours. Steps i) and ii) of the method of the invention may thus be carried out quickly, in particular without having to wait for fungal cells or the like to provide the first fibers.

In an embodiment, step iii) is carried out and completed within 72 hours from the start of step ii), preferably within 5 hours. In particular in combination with the previous embodiment, this may allow the non-woven textile to be produced within 4 days.

According to a second, the invention provides a non-woven textile, preferably obtained using the method of the invention, comprising biobased first fibres and reinforcing second fibres, wherein said first and second fibers are irreversibly embedded in a matrix comprising a plasticizer; wherein the biobased first fibers are fibers derived from a micro-organism that has been cultured in a liquid culture medium, and wherein the second fibers have an average length that is at least 10x longer than the average length of the first fibers.

Besides the plasticizer, the matrix typically further comprises some moisture, e.g. from a dispersion medium that may have been in accordance with step i) of the claimed method.

When the non-woven textile is obtained using the method of the invention, preferably the non-woven textile has a seamless circumferential surface.

In an embodiment said plasticizer comprises an amorphous matrix comprising a hydroxic acid and a polyol.

In an preferred embodiment, the first fibers comprise 20 - 80 % weight of the non-woven textile; the second fibers comprise 1 - 40 % weight of the non-woven textile; and the plasticizer comprises 5 - 50 % weight of the non-woven textile; wherein the combined % weight of the first fibers, the second fibers and the plasticizer is at least 65% of the weight of the non-woven textile, preferably at least 80%; and wherein the %weight of the second fibers is less than the %weight of the first fibers.

In an embodiment oil droplets and/or fatty droplets are embedded in the matrix, said droplets having a maximum diameter in the range of 1 µm to 20 µm. For instance, the oil droplets may comprise a drying oil or a non drying oil. Optionally, a siccative is included in the matrix as well.

According to a third aspect, the present invention provides a shaped seamless garment, accessory or footwear to be worn, or any other three dimensional seamless non-woven textile product, comprising the non-woven textile of the second aspect, and/or a non-woven textile produced in accordance with the first aspect of the invention. Thus, the invention provides a garment, accessory, footwear or other product that is seamless.

The invention will now be illustrated with reference to the example section below, and with reference to the drawing wherein
Fig 1. shows a schematic representation of a cross section of a non-woven textile;
Figs. 2A-2C respectively show a schematic representation of another embodiment of a non-woven textile according to the invention, and a first detail and a second detail thereof;
Figs. 3A-3C respectively show a schematic representation of yet another embodiment of a non-woven textile according to the invention, and a first detail and a second detail thereof; and
Fig. 4 shows an embodiment of a non-woven textile in the form of a bag that has a three-dimensional non-planar shape and which has been manufactured according to the method of the invention.

Figure 1 shows a schematic representation of a cross section of a non-woven textile 100 comprising first fibers 110 and second fibers 120 produced according to the invention. The first fibers 110 were derived from cultured mycelium, and dispersed in a dispersion medium. A first layer of the dispersion comprising first fibers 110 was applied to a support and second fibers 120 were added to the layer of the dispersion. A second layer of the dispersion was added on top of the first layer of the dispersion, and dispersion medium was eliminated by evaporation at room temperature. In the resulting non-woven textile, the first fibers 110 present as a continuous web, without distinguishable borders between the first fibers 110 applied in the first layer of the dispersion, and the first fibers 110 applied in the second layer of the dispersion. The second fibers 120 are embedded in the continuous web of first fibers 110.

In order to produce the non-woven textile, fungal biomass in the form of Schizophyllum commune mycelium from the group of basidiomycota, was grown in standard Malt extract in a 1 liter Duran Erlenmeyer. The growth procedure followed standard culture procedures at 30°C and shaking at 200 rpm. Mycelium was harvested by means of Buchner filtration. Citric acid and sorbitol were pre-mixed with water, and subsequently added to the harvested mycelium comprised and the remainder of the growth medium, forming the dispersion comprising the first fibers.

In step a), a first layer of the dispersion was applied on a mold by spraying the dispersion on a solid and 3D shaped support surface with a spraying machine used for spraying paint. In step b), the dispersion medium was eliminated by means of evaporation at room temperature. The dispersion medium was evaporated until a web of mycelium (MYC) dry to the touch was formed at the support.

Steps a) an b) were repeated once more. Subsequently, in step c) a further layer of dispersion was applied on top of the web. In step d), individual second fibers, such as polyamide (PA) 100 dtex, or carded rayon (CV) 28 dtex were applied by flocking with a FK1-PRO onto the web, while carded flax (LI) was applied by hand. For example, the rayon fibers were 12 mm long with a circular circumferential surface spanning in between two ends. In a plane projected parallel to a face of the second web, the area of the first fibers covered by the second fibers was 30-50%.

Steps a), b), c) and d) were then repeated twice, and finally steps a) and b) were performed once.

The resulting non-woven textile was taken from the mold. In a cross section of the non-woven textile, no individual webs or first fibers were distinguishable, but rather presented as one single web of first fibers with the second fibers embedded within the single web of first fibers. The second fibers do not present as distinct and continuous layers in the non-woven textile. Instead, the second fibers applied in the same step are substantially aligned to either outside surface of the non-woven textile, and may be in contact with each other and may be aligned as well as crossing each other under diverse angles.

From each non-woven textile, the extension and the peak force were measured in order to evaluate the effect of the second fibers on the non-woven textile. The extension and peak force were measured according to EN13934-01, with this exception that the dimensions of the tested samples were 4 x 4 cm. Experiments were performed either as single experiments or in duplicate. As a control, a non-woven textile of pure mycelium was used.

**Table 1 shows the effect of various second fibers on the extension and peak force**

| **Sample** | **Sample thickness (mm)** | **Peak distance (mm)** | **Extension (%)** | **Peak force (N)** |
|---|---|---|---|---|
| 1a. Mycelium pure | 0.26 - 0.45 | 4.7 | 12 | 14 |
| 1b. Mycelium pure | 0.39 - 0.44 | 6.2 | 16 | 12 |

| **Average** | | | **14** | **13** |
|---|---|---|---|---|
| 2a. MYC/MYC PA 100 dtex, sprayed | 0.44 - 0.49 | 4.1 | 10 | 45 |
| 2b. MYC/MYC PA 100 dtex, sprayed | 0.47 - 0.48 | 5.3 | 13 | 70 |

| **Average** | | | **12** | **58** |
|---|---|---|---|---|
| 3a. MYC/MYC PA 100 dtex, sprayed | 0.85 - 0.88 | 7.7 | 19 | 61 |
| 3b. MYC/MYC PA 100 dtex, sprayed | 0.76 - 0.87 | 8.9 | 22 | 69 |

| **Average** | | | **21** | **65** |
|---|---|---|---|---|
| 4. MYC/LI carded, sprayed | 0.59 - 0.66 | 5.8 | 14 | 88 |
| 5. MYC/CV 28 dtex, sprayed | 0.31- 0.33 | 5.3 | 13 | 21 |

The addition of second fiber resulted in a peak force which was 1.6 - 6.8 x higher than non-woven textile from pure mycelium, indicating that the addition of the second fiber confers strength to the non-woven textile.

Furthermore, the skin feel of the non-woven textiles was evaluated by a panel of 5 people, who independently assessed the skin feel of the non-woven textiles comprising second fibers to be the same as the skin feel of the non-woven textile from pure mycelium.

Fig. 2A shows a schematic representation of a cross section of another non-woven textile 200 comprising first biobased fibers 210 and second reinforcing fibers 220 produced according to the invention. In the cross-section, the textile 200 has an upper outer surface 201, and a lower outer surface 202, between the first and second fibers are arranged. Though in the example shown, the first and second fibers are embedded in a single fused layer, it will be appreciated that instead the non-woven textile may comprise a stack of multiple fused layers of first and second fibers. The first fibers form a web that is reinforced by the second fibers.

Fig. 2B shows a detail of portion II-B of Fig. 2A, in which the first fibers 210 and a second fibers 220 are shown in greater detail. As can be seen, the first fibers are smaller by orders of magnitude that the second fibers 220. In the example shown, the first fibers 210, which are shown in even greater detail in Fig. 2C, have an average diameter of about 2 µm, whereas the second fibers 220 have an average diameter of about 100 µm. As can be seen, the larger second fibers 220 are substantially aligned with the upper and lower outer surfaces 201, 202 such that their center lines are substantially parallel to these surfaces 201, 202. The first fibers 210, which are much smaller, are oriented substantially randomly and are not substantially aligned with the first and second outer surfaces.

The first and second fibers are embedded in a matrix 230 comprising a plasticizer, which, besides helping to hold the first and second fibers substantially in place, also provides the non-woven textile with a degree of flexibility allowing it to be bend or folded, without breaking the non-woven textile. The plasticizer preferably comprises 5 - 50 %, preferably 15-30% by weight of the finished non-woven textile, and preferably comprises a mixture of a polyol, such as sorbitol, and an alpha hydroxy acid, such as citric acid.

Fig.3A shows a schematic representation of a cross section of yet another non-woven textile 300 according to the invention. In addition to biobased first fibers 310 and second reinforcement fibers 320 that are embedded in a matrix 330 which comprises a plasticizer and optionally any remaining dispersing medium. Further shown are oil droplets 340 which are embedded in the matrix 330 and can have various sizes, with the maximum diameter of each oil drop typically in the range of between 1 µm and 20 µm. The oil droplets 340 may be used for a delayed control or controlled release of beneficial fat-soluable components, and in the present example comprise oil of aloe vera, which provides a nice scent. The oil droplets 340 typically have an average diameter which is larger than the average length of the first fibers, e.g. at least 5 times larger than an average length of the first fibers 310.

Fig. 4 shows a perspective line drawing of a non-woven textile 400 according to the invention, formed as a non-planar shape, here in the form of a hand-bag. The non-woven textile 400 has been manufactured by applying a layer of a dispersion onto a non-planar support (not shown) that has positive shape of the non-woven textile 400. The layer is typically applied either by spraying the dispersion onto a non-planar 3D-surface of the support, and/or by using a brush to apply the dispersion to the support. After the layer of dispersion, which comprises a dispersion medium, first biobased fibers as well as a plasticizer, was applied, a layer of reinforcing second fibers were deposited onto the layer of dispersion, after which the two layers were allowed to dry to form the non-woven textile 400. The non-woven textile 400 comprises a circumferential surface 401, which is provided with ridges 402, as well as with dimples 403. In the present example, the layer of dispersion was applied on a flexible support, and after the second fibers were applied and the dispersion medium was eliminated to form the non-woven textile 400, the flexible support was collapsed and removed from the inner side of the textile 400. It will be apparent to the person skilled in the art that additionally or instead one or more supports can be used for creating a positive or negative shape, e.g. in ways similar to casting molds used in casting processes, to allow easy removal of the non-woven textile from the support(s). By using one or more supports, the final product may be produced free from stitches or glued seams or the like.

## Claims

1. A method for producing a non-woven textile (100), wherein said method comprises the following steps:
i) applying a layer of a dispersion comprising dispersion medium and biobased first fibers (110) on a support, wherein the biobased first fibers (110) are fibers derived from a micro-organism cultured in a liquid culture medium, and wherein, prior to said applying, a plasticizer has been added to the dispersion;
ii) depositing reinforcing second fibers (120) on the layer of the dispersion, wherein the reinforcing second fibers (120) are separate fibers which are not part of a fabric, and wherein the second fibers have an average length that is at least 10x longer than the average length of the first fibers; and
iii) eliminating the dispersion medium to form the non-woven textile (100) comprising a web of biobased first fibers (110).

2. The method according to claim 1, wherein the layer of the dispersion in step i) is applied by spraying,
the method preferably further comprising removing the non-woven textile from the support.

3. The method according to any of the preceding claims,
wherein the plasticizer is a sugar alcohol, a polyol, polyolester and/or an alpha hydroxy acid, or a combination thereof, preferably wherein the plasticizer comprises a combination of sorbitol and citric acid; or
wherein said plasticizer comprises one or more of glycols, glyceryl triacetate, polymeric polyols, quillaia, honey, molasses, aloe vera, castor oil, glycerides, triglycerides and other mineral or organic oil.

4. The method according to any of the preceding claims, wherein step i) is preceded by a step comprising
- supplying a dispersion of biobased first fibers (110), said first fibers (110) being dispersed in a dispersion medium, and
- eliminating at least part of said dispersion medium so as to form a web on the support; which step is performed at least once, and step i) comprises applying the layer of dispersion onto the web.

5. The method according to any of the preceding claims, wherein the method further comprises between steps ii) and iii) a step of applying a further layer of a further dispersion on top of the layer of the dispersion, said further dispersion comprising further dispersion medium and biobased third fibers.

6. The method according to claim 1, wherein the biobased first fibers (110) are in the form of a biological material chosen from: fungal mycelium, yeast, algae, bacteria, cultured animal or plant cells, fibers derived from animal and/or plant cells cultured in a liquid culture medium.

7. The method according to any of the preceding claims, wherein the second fibers (120) are selected from natural fibers, regenerated fibers, recycled fibers, synthetic fibers, or any combination thereof, preferably wherein the second fibers (120) are hydrophilic.

8. The method according to any of the preceding claims, wherein the concentration of first fibers in the dispersion is at least 0.1% w/v, preferably at least 5% w/v, more preferably at least 10% w/v and most preferably at least 15% w/v.

9. The method according to any of the preceding claims, wherein the dispersion further comprises oil droplets.

10. The method according to any of the preceding claims, wherein the method comprises a step of applying and adhering at least one component to the web,
preferably wherein said at least one component is selected from the group of led-lighting, sensors, RFID tags or NFC chips, or embellishments, for example sequins, beads, cord, appliqué and lace;
wherein said at least one component is embedded in the non-woven textile without gluing or sewing the component to the non-woven textile.

11. The method according to any of the preceding claims, wherein the method further comprises a dyeing step, preferably wherein dye or pigment is co-applied with at least one chosen from the first and second fibers, more preferably wherein no liquid other than the dispersion is used to apply the dye and/or pigment.

12. The method according to any of the preceding claims, wherein the support has a three-dimensional non-flat surface.

13. Non-woven textile, preferably obtained by a method according to any one of the preceding claims 1-12, comprising biobased first fibres and reinforcing second fibres, wherein said first and second fibers are irreversibly embedded in an amorphous matrix comprising plasticizer;
wherein the biobased first fibers (110) are fibers derived from a micro-organism that has been cultured in a liquid culture medium, and
wherein the second fibers have an average length that is at least 10x longer than the average length of the first fibers.

14. Non-woven textile according to claim 13, wherein said plasticizer is formed from an alpha hydroxy acid and a polyol.

15. Non-woven textile according to claim 13 or 14, wherein
the first fibers comprise 20 - 80 % weight of the non-woven textile;
the second fibers comprise 1 - 40 % weight of the non-woven textile; and
the plasticizer comprises 5 - 50 % weight of the non-woven textile,
wherein the combined % weight of the first fibers, the second fibers and the plasticizer is at least 65% of the weight of the non-woven textile, preferably at least 80%; and
wherein the %weight of the second fibers is less than the %weight of the first fibers.

16. Non-woven textile according to any one of claims 13 - 15, wherein oil droplets and/or fatty droplets are embedded in the matrix, said droplets having a maximum diameter in the range of 1 µm to 20 µm.

17. Shaped seamless garment, accessory or footwear to be worn, or any other three dimensional seamless non-woven textile product, comprising the non-woven textile according to any of claims 13 - 16.

## Patentansprüche

1. Verfahren zur Herstellung eines Vliesstoffs (100), wobei das Verfahren die folgenden Schritte umfasst:
i) Aufbringen einer Schicht einer Dispersion, die Dispersionsmedium und erste Fasern auf Biobasis (110) umfasst, auf einen Träger, wobei die ersten Fasern auf Biobasis (110) Fasern sind, die von einem in einem flüssigen Kulturmedium kultivierten Mikroorganismus abgeleitet sind, und wobei vor dem Aufbringen ein Weichmacher zu der Dispersion zugegeben worden ist;
ii) Abscheiden von verstärkenden zweiten Fasern (120) auf die Schicht der Dispersion, wobei die verstärkenden zweiten Fasern (120) gesonderte Fasern sind, die nicht Teil eines Gewebes sind, und wobei die zweiten Fasern eine mittlere Länge aufweisen, die wenigstens 10x länger als die mittlere Länge der ersten Fasern ist; und
iii) Entfernen des Dispersionsmediums, um den Vliesstoff (100) zu bilden, der eine Bahn von ersten Fasern auf Biobasis (110) umfasst.

2. Verfahren nach Anspruch 1, wobei die Schicht der Dispersion bei Schritt i) durch Sprühen aufgebracht wird,
wobei das Verfahren vorzugsweise ferner Entfernen des Vliesstoffs von dem Träger umfasst.

3. Verfahren nach einem der vorstehenden Ansprüche,
wobei der Weichmacher ein Zuckeralkohol, ein Polyol, Polyolester und/oder eine alpha-Hydroxysäure oder eine Kombination davon ist, wobei der Weichmacher vorzugsweise eine Kombination von Sorbit und Zitronensäure umfasst; oder
wobei der Weichmacher eines oder mehrere von Glycolen, Glyceryltriacetat, polymeren Polyolen, Quillaia, Honig, Melasse, Aloe vera, Rizinusöl, Glyceriden, Triglyceriden und anderem Mineral- oder organischem Öl umfasst.

4. Verfahren nach einem der vorstehenden Ansprüche, wobei Schritt i) ein Schritt vorangeht, umfassend
- Zuführen einer Dispersion von ersten Fasern auf Biobasis (110), wobei die ersten Fasern (110) in einem Dispersionsmedium dispergiert sind, und
- Entfernen wenigstens eines Teils des Dispersionsmediums, um eine Bahn auf dem Träger zu bilden; wobei der Schritt wenigstens einmal durchgeführt wird und Schritt i) Aufbringen der Dispersionsschicht auf die Bahn umfasst.

5. Verfahren nach einem der vorstehenden Ansprüche, wobei das Verfahren ferner zwischen Schritten ii) und iii) einen Schritt des Aufbringens einer weiteren Schicht einer weiteren Dispersion auf die Schicht der Dispersion umfasst, wobei die weitere Dispersion weiteres Dispersionsmedium und dritte Fasern auf Biobasis umfasst.

6. Verfahren nach Anspruch 1, wobei die ersten Fasern auf Biobasis (110) in der Form eines biologischen Materials vorliegen, das ausgewählt ist aus: Pilzmyzel, Hefe, Algen, Bakterien, kultivierten Tier- oder Pflanzenzellen, von in einem flüssigen Kulturmedium kultivierten Tier- und/oder Pflanzenzellen abgeleiteten Fasern.

7. Verfahren nach einem der vorstehenden Ansprüche, wobei die zweiten Fasern (120) ausgewählt sind aus natürlichen Fasern, regenerierten Fasern, recycelten Fasern, synthetischen Fasern oder einer beliebigen Kombination davon, wobei die zweiten Fasern (120) vorzugsweise hydrophil sind.

8. Verfahren nach einem der vorstehenden Ansprüche, wobei die Konzentration der ersten Fasern in der Dispersion wenigstens 0,1 % w/v, vorzugsweise wenigstens 5 % w/v, bevorzugter wenigstens 10 % w/v und höchst bevorzugt wenigstens 15 % w/v beträgt.

9. Verfahren nach einem der vorstehenden Ansprüche, wobei die Dispersion ferner Öltröpfchen umfasst.

10. Verfahren nach einem der vorstehenden Ansprüche, wobei das Verfahren einen Schritt des Aufbringens und Anhaftens wenigstens einer Komponente an die Bahn umfasst,
wobei vorzugsweise die wenigstens eine Komponente ausgewählt ist aus der Gruppe von LED-Beleuchtung, Sensoren, RFID-Tags und NFC-Chips, und Verzierungen, beispielsweise Pailletten, Perlen, Kord, Applikation und Spitze;
wobei die wenigstens eine Komponente ohne Verkleben oder Vernähen der Komponente mit dem Vliesstoff in dem Vliesstoff eingebettet ist.

11. Verfahren nach einem der vorstehenden Ansprüche, wobei das Verfahren ferner einen Färbeschritt umfasst, wobei vorzugsweise Farbstoff oder Pigment gemeinsam mit wenigstens einer ausgewählt aus der ersten und der zweiten Faser aufgebracht wird, wobei bevorzugter keine andere Flüssigkeit als die Dispersion zum Aufbringen des Farbstoffs und/oder Pigments verwendet wird.

12. Verfahren nach einem der vorstehenden Ansprüche, wobei der Träger eine dreidimensionale nichtflache Oberfläche aufweist.

13. Vliesstoff, vorzugsweise erhalten durch ein Verfahren nach einem der vorstehenden Ansprüche 1-12, umfassend erste Fasern auf Biobasis und verstärkende zweite Fasern, wobei die ersten und zweiten Fasern irreversibel in eine amorphe Matrix, die Weichmacher umfasst, eingebettet sind;
wobei die ersten Fasern auf Biobasis (110) Fasern sind, die von einem Mikroorganismus abgeleitet sind, der in einem flüssigen Kulturmedium kultiviert worden ist, und
wobei die zweiten Fasern eine mittlere Länge aufweisen, die wenigstens 10x länger als die mittlere Länge der ersten Fasern ist.

14. Vliesstoff nach Anspruch 13, wobei der Weichmacher aus einer alpha-Hydroxysäure und einem Polyol gebildet ist.

15. Vliesstoff nach Anspruch 13 oder 14, wobei
die ersten Fasern 20-80 Gew.-% des Vliesstoffs umfassen;
die zweiten Fasern 1-40 Gew.-% des Vliesstoffs umfassen; und
der Weichmacher 5-50 Gew.-% des Vliesstoffs umfasst,
wobei die kombinierten Gew.-% der ersten Fasern, der zweiten Fasern und des Weichmachers wenigstens 65 % des Gewichts des Vliesstoffs, vorzugsweise wenigstens 80 %, betragen; und
wobei die Gew.-% der zweiten Fasern kleiner als die Gew.-% der ersten Fasern sind.

16. Vliesstoff nach einem der Ansprüche 13-15, wobei Öltröpfchen und/oder Fetttröpfchen in die Matrix eingebettet sind, wobei die Tröpfchen einen maximalen Durchmesser in dem Bereich von 1 µm bis 20 µm aufweisen.

17. Geformtes nahtloses Kleidungsstück, Accessoire oder Schuhwerk zum Tragen oder ein beliebiges anderes dreidimensionales nahtloses Vliesstoffprodukt, das den Vliesstoff nach einem der Ansprüche 13-16 umfasst.

## Revendications

1. Procédé de production d'un textile non tissé (100), dans lequel ledit procédé comprend les étapes suivantes:
i) application d'une couche d'une dispersion comprenant un milieu de dispersion et des premières fibres biosourcées (110) sur un support, dans lequel les premières fibres biosourcées (110) sont des fibres dérivées d'un micro-organisme cultivé dans un milieu de culture liquide, et dans lequel, avant ladite application, un plastifiant a été ajouté à la dispersion;
ii) dépôt de secondes fibres de renforcement (120) sur la couche de la dispersion, dans lequel les secondes fibres de renforcement (120) sont des fibres distinctes qui ne font pas partie d'un tissu, et dans lequel les secondes fibres ont une longueur moyenne qui est au moins 10 fois plus longue que la longueur moyenne des premières fibres; et
iii) élimination du milieu de dispersion pour former le textile non tissé (100) comprenant une bande de premières fibres biosourcées (110).

2. Procédé selon la revendication 1, dans lequel la couche de la dispersion dans l'étape i) est appliquée par pulvérisation,
de préférence, le procédé comprend en outre l'élimination du textile non tissé du support.

3. Procédé selon l'une quelconque des revendications précédentes,
dans lequel le plastifiant est un alcool de sucre, un polyol, un polyolester et/ou un alpha hydroxy acide, ou une combinaison de ceux-ci, de préférence dans lequel le plastifiant comprend une combinaison de sorbitol et d'acide citrique; ou
dans lequel ledit plastifiant comprend un ou plusieurs parmi des glycols, le triacétate de glycéryle, des polyols polymères, le quillaia, un miel, une mélasse, de l'aloe vera, une huile de ricin, des glycérides, des triglycérides et une autre huile minérale ou organique.

4. Procédé selon l'une quelconque des revendications précédentes, dans lequel l'étape i) est précédée d'une étape comprenant
- la fourniture d'une dispersion de premières fibres biosourcées (110), lesdites premières fibres (110) étant dispersées dans un milieu de dispersion, et
- l'élimination d'au moins une partie dudit milieu de dispersion pour former une bande sur le support; laquelle étape étant effectuée au moins une fois, et l'étape 1) comprend l'application de la couche de dispersion sur la bande.

5. Procédé selon l'une quelconque des revendications précédentes, dans lequel le procédé comprend en outre, entre les étapes ii) et iii), une étape d'application d'une couche supplémentaire d'une dispersion supplémentaire au-dessus de la couche de la dispersion, ladite dispersion supplémentaire comprenant un milieu de dispersion supplémentaire et des troisièmes fibres biosourcées.

6. Procédé selon la revendication 1, dans lequel les premières fibres biosourcées (110) sont sous la forme d'un matériau biologique choisi parmi : mycélium fongique, levure, algues, bactéries, cellules animales ou végétales cultivées, fibres dérivées de cellules animales et/ou végétales cultivées dans un milieu de culture liquide.

7. Procédé selon l'une quelconque des revendications précédentes, dans lequel les secondes fibres (120) sont choisies parmi des fibres naturelles, des fibres régénérées, des fibres recyclées, des fibres synthétiques ou toute combinaison de celles-ci, de préférence dans lequel les secondes fibres (120) sont hydrophiles.

8. Procédé selon l'une quelconque des revendications précédentes, dans lequel la concentration des premières fibres dans la dispersion est d'au moins 0,1 % en p/v, de préférence d'au moins 5 % en p/v, plus préférablement d'au moins 10 % en p/v et le plus préférablement d'au moins 15 % en p/v.

9. Procédé selon l'une quelconque des revendications précédentes, dans lequel la dispersion comprend en outre des gouttelettes d'huile.

10. Procédé selon l'une quelconque des revendications précédentes, dans lequel le procédé comprend une étape d'application et de collage d'au moins un composant sur la bande,
de préférence, dans lequel ledit au moins un composant est choisi dans le groupe d'un éclairage led, des capteurs, des étiquettes RFID ou des puces NFC, ou des embellissements, par exemple des paillettes, des perles, un cordon, une applique et une dentelle;
dans lequel ledit au moins un composant est incorporé dans le textile non tissé sans coller ou coudre le composant au textile non tissé.

11. Procédé selon l'une quelconque des revendications précédentes, dans lequel le procédé comprend en outre une étape de teinture, de préférence dans lequel un colorant ou un pigment est co-appliqué avec au moins une fibre choisie parmi les premières et secondes fibres, plus préférablement dans lequel aucun liquide autre que la dispersion n'est utilisé pour appliquer le colorant et/ou le pigment.

12. Procédé selon l'une quelconque des revendications précédentes, dans lequel le support a une surface tridimensionnelle non plate.

13. Textile non tissé, de préférence obtenu par un procédé selon l'une quelconque des revendications 1 à 12 précédentes, comprenant des premières fibres biosourcées et des secondes fibres de renforcement, dans lequel lesdites premières et secondes fibres sont incorporées de manière irréversible dans une matrice amorphe comprenant un plastifiant;
dans lequel les premières fibres biosourcées (110) sont des fibres dérivées d'un micro-organisme qui a été cultivé dans un milieu de culture liquide, et
les secondes fibres ont une longueur moyenne qui est au moins 10 fois plus longue que la longueur moyenne des premières fibres.

14. Textile non tissé selon la revendication 13, dans lequel ledit plastifiant est formé à partir d'un alpha hydroxy acide et d'un polyol.

15. Textile non tissé selon la revendication 13 ou 14, dans lequel
les premières fibres constituent 20 à 80 % en poids du textile non tissé;
les secondes fibres constituent 1 à 40 % en poids du textile non tissé; et
le plastifiant constitue 5 à 50 % en poids du textile non tissé,
dans lequel le pourcentage en poids combiné des premières fibres, des secondes fibres et du plastifiant est au moins 65 % du poids du textile non tissé, de préférence au moins 80 %; et
dans lequel le pourcentage en poids des secondes fibres est inférieur au pourcentage en poids des premières fibres.

16. Textile non tissé selon l'une quelconque des revendications 13 à 15, dans lequel des gouttelettes d'huile et/ou des gouttelettes grasses sont incorporées dans la matrice, lesdites gouttelettes ayant un diamètre maximal dans la plage de 1 µm à 20 µm.

17. Vêtement, accessoire ou chaussure façonné(e) sans couture à porter, ou tout autre produit de textile non tissé sans couture tridimensionnel, comprenant le textile non tissé selon l'une quelconque des revendications 13 à 16.
